

# United States Patent

[11] 3,627,672

[72] Inventors **James R. Kittrell**  
**El Cerrito;**  
**Richard C. Robinson, San Rafael, both of**  
**Calif.**  
[21] Appl. No. **862,036**  
[22] Filed **Sept. 29, 1969**  
[45] Patented **Dec. 14, 1971**  
[73] Assignee **Chevron Research Company**  
**San Francisco, Calif.**

[54] **CATALYTIC HYDROGENATION WITH METAL**  
**PHOSPHATE-CONTAINING CATALYSTS**  
3 Claims, No Drawings

[52] U.S. Cl..... **208/143,**  
                          260/667, 252/437, 252/455  
[51] Int. Cl..... **C07c 5/10,**  
                          C10g 23/02  
[50] Field of Search..... **208/143;**  
                          260/667; 252/437, 455

[56]

## References Cited

### UNITED STATES PATENTS

|           |        |                    |         |
|-----------|--------|--------------------|---------|
| 3,147,210 | 9/1964 | Hass et al.....    | 208/210 |
| 3,175,014 | 3/1965 | Ballard et al..... | 260/667 |
| 3,186,935 | 6/1965 | Vaeil .....        | 208/59  |
| 3,493,517 | 2/1970 | Jaffee .....       | 208/254 |
| 3,516,927 | 6/1970 | Jaffee .....       | 208/143 |

Primary Examiner—Herbert Levine

Attorneys—A. L. Snow, F. E. Johnston, C. J. Tonkin and R. H. Davies

**ABSTRACT:** Aromatics hydrogenation process using a catalyst having a particle density greater than 1.4 g./cc., comprising alumina, a component selected from nickel and compounds thereof and cobalt and compounds thereof, a component selected from molybdenum and compounds thereof, and a component selected from titanium phosphate and zirconium phosphate.

## CATALYTIC HYDROGENATION WITH METAL PHOSPHATE-CONTAINING CATALYSTS

## INTRODUCTION

This application relates to hydrogenation of aromatic hydrocarbons.

## PRIOR ART

It is known that many hydrocarbon stocks such as jet fuels, kerosene, furnaces oils, lubricating oils, etc., can be upgraded by partial or completed hydrogenation of the aromatic constituents thereof.

Aromatic hydrogenation results in improved burning characteristics for many fuels. For example, in the case of jet fuels, desirably increases in smoke points can be obtained by hydrogenation of the aromatics contained in the fuels to the corresponding naphthenes, which have higher heats of combustion.

Commercial hydrofining processes directed to the removal of contaminants such as sulfur and nitrogen from hydrocarbon feedstocks inherently accomplish hydrogenation of olefin constituents of the feedstocks; however, these processes accomplish little or no hydrogenation or aromatics content in the feedstocks.

Aromatics hydrogenation processes are well known. Prior art hydrogenation catalysts generally comprise platinum on alumina, occasionally with a minor proportion of added halogen. Various other group VIII metals, such as nickel, cobalt and iron, as well as other metals of the platinum group, deposited on alumina or other suitable carriers also have been employed. The prior art processes have been carried out at temperatures within the range 300° to 900° F., pressures within the range 1,9000 to 5,000 p.s.i.g., and liquid hourly space velocities in the range 0.1 to 20, in the presence of 2,500 to 25,000 standard cubic feet of hydrogen per barrel of charged material. Generally, low-catalyst densities are desirably for platinum hydrogenation catalysts of the prior art, as exemplified by U.S. Pat. No. 3,432,565.

Conventional aromatics hydrogenation processes are disclosed in the following representative U.S. Pat. Nos.

2,967,204  
3,012,961  
3,077,733  
3,147,210  
3,172,833  
3,432,565  
3,432,565

Conventional aromatics hydrogenation catalysts, particularly catalysts containing group VIII noble metals, are sulfur-sensitive, and the presence of organic sulfur compounds in the feed exerts a deleterious effect on the hydrogenation activity of these catalysts. The sulfur sensitivity of the group VIII noble metal hydrogenation catalysts is particularly discussed in the aforesaid U.S. Pats. Nos. 3,147,210 and 3,186,935.

In view of the importance of aromatics hydrogenation for improving the burning characteristics of man aromatics-containing hydrocarbon feedstocks, there is a continuing search for improved processes for accomplishing the desired hydrogenation, particularly processes using aromatics hydrogenation catalysts having higher aromatics hydrogenation activities and/or lower fouling rates, that is, higher stabilities.

## OBJECTS

In view of the foregoing, it is an object of the present invention to provide an improved aromatics hydrogenation process employing a catalyst of high-activity and stability which permits the process to be operated at reasonable temperatures for long periods of time. It is a further object of the present invention to provide an aromatics hydrogenation process using a catalyst which contains less costly constituents than the conventional group VIII noble metal hydrogenation catalysts, and which is more sulfur-tolerant than those conventional catalysts.

## STATEMENT OF INVENTION

In accordance with the present invention, there is provided an aromatics hydrogenation process which comprises contacting an aromatics-containing hydrocarbon feedstock under aromatics hydrogenation conditions with hydrogen and a catalyst comprising alumina, a component selected from nickel and compounds thereof and cobalt and compounds thereof, a component selected from molybdenum and compounds thereof and a component selected from titanium phosphate and zirconium phosphate, the particle density of said catalyst exceeding 1.4 g./cc. In preferred embodiment of the process of the present invention, the catalyst used therein contains 0.5 to 20 weight percent, preferably 0.5 to 5 weight percent, natural or synthetic clay, or natural or synthetic zeolite, based on the total catalyst. Specific calcination conditions can also achieve such particle densities.

The aromatics hydrogenation conditions used in the process of the present invention are conventional conditions as discussed below.

## CATALYST ACTIVITIES

The activity of any catalyst can be described by the rate constant of the reaction of a reference catalyst temperature. For aromatics hydrogenation, said rate constant may be written:

$$k = LHSV \ln \left( \frac{A_f - A_e}{A_p - A_e} \right)$$

where  $k$  is the rate constant, LHSV is liquid hourly space velocity (note exact definitions in the following paragraph),  $A_f$  is the aromatic content of the feed,  $A_p$  is the aromatic content of the hydrogenated product, and  $A_e$  is the aromatic content which would be obtained in the product had the reaction proceeded to equilibrium.

A variety of definitions for space velocities are usable in the above expression. Because of variations in reactor bed packing and the relation of the surface area, and therefore catalytically active sites to a weight of catalyst (usually given as square meters/gram), the most significant space velocity is based on weight measures:

$$(LHSV)_w = \frac{\text{Feed rate, grams/hour}}{\text{Catalyst weight, grams}}$$

It is thus most accurate to rank catalysts using activities calculated on a weight space velocity. However, commercial applications of kerosene hydrogenation require minimizing the volume of the catalyst bed in order to minimize capital investment. Hence, a space velocity definition of commercial interest is based on volume measures:

$$(LHSV)_v = \frac{\text{Feed rate, cc./hour}}{\text{Catalyst volume, cc.}}$$

Therefore, a ranking of catalyst activities for commercial use must be calculated on volumetric space velocities.

If all catalysts exhibited the same bulk density when packed into a reactor, of course rankings of catalysts on these two bases would be fully equivalent. However, variation in catalyst preparations techniques can vary either the packing factor or the particle density of the catalysts, thus changing these rankings. For example, Kouwenhoven, et al. in U.S. Pat. No. 3,432,565 have demonstrated that low-density hydrogenation catalysts exhibit highest activities if the catalyst is comprised of group VIII metals on alumina. The present invention is directed to an aromatic hydrogenation process using a high-density catalyst comprising alumina, a component selected from nickel and compounds thereof and cobalt and compounds thereof, a component selected from molybdenum and compounds thereof, and a component selected from titanium phosphate and zirconium phosphate.

## FEEDSTOCKS

Hydrocarbon feedstocks which may be used to advantage in the process of the present invention include a wide range of aromatics-containing hydrocarbon feedstocks, for example light and heavy straight run gas oils, light and heavy cracked cycle oils, and various aromatic extracts.

The hydrocarbon feedstock will contain 5 to 95 percent preferably 20 to 80 percent, aromatics.

Cracked stocks may be obtained from thermal or catalytic cracking of various stocks, including those obtained from petroleum, gilsonite, shale and coal tar.

The organic nitrogen and organic sulfur contents of the hydrocarbon feedstocks each may range from a few parts per million to several weight percent. If desired, the feedstocks may be treated in a conventional hydrofining step to reduce the sulfur and nitrogen contents thereof, prior to being hydrogenated in accordance with the process of the present invention.

## HYDROGENATION CONDITIONS

The process of the present invention may be carried out at conventional hydrogenation conditions, for example at a temperature in the range 400° to 900° F., a pressure in the range 500 p.s.i.g., and a liquid hourly space velocity in the range 0.2 to 20, and in presence of 1,000 to 20,000 standard cubic feet of hydrogen per barrel of charged material.

The process of the present invention may be carried out at any desired combination of conditions within the foregoing ranges with produce a desired degree of aromatics hydrogenation. Desirably, a combination of conditions is selected which will result in hydrogenation of more than 50 volume percent and preferably more than 90 volume percent of the aromatics present in the feedstock.

## CATALYST CONSTITUENTS AND AMOUNTS THEREOF

The catalyst used in the process of the present invention will contain the following constituents in the indicated amounts:

|                                      | Wt. %, calculated as metal |
|--------------------------------------|----------------------------|
| Ni or Co, generally as NiO or CoO    | 1-10                       |
| Mo, generally as MoO <sub>3</sub>    | 5-25                       |
| TiO <sub>2</sub> or ZrO <sub>2</sub> | 5-20                       |
| P <sub>2</sub> O <sub>5</sub>        | 3-15                       |
| Al <sub>2</sub> O <sub>3</sub>       | at least 20                |
| Clay and/or zeolite                  | 0-20                       |

Additionally, the catalyst may contain combined fluorine, in an amount of 0-10 weight percent.

When the catalyst used in the process of the present invention contains titanium and no zirconium, the titanium:phosphate atomic ratio will be greater than 1:1. When the catalyst used in the process of the present invention contains zirconium and no titanium, the zirconium:phosphate ratio will be greater than 1:2.

## CATALYST PREPARATIONS

The catalyst used in the process of the present invention conveniently may be prepared by such methods as impregnation of an alumina or silica-alumina support with salts of the desired hydrogenation component, or cogelation of all components, with the latter method being preferred. When the catalyst is cogelled, the necessary form for the catalyst used in the process of the present invention will be obtained, that is, one in which the titanium or zirconium is combined with the phosphorus as discrete particles of titanium phosphate or zirconium phosphate, dispersed through a carrier, or matrix, of the other catalyst components. The necessary high densities can be achieved by including in the catalyst a natural or synthetic clay, or a crystalline zeolitic molecular sieve, and/or by drying the cogel thoroughly and calcining the catalyst with high rates of dry air.

## EXAMPLES

The following examples will serve to further illustrate the practice of the present invention and its advantages.

## EXAMPLE 1

A catalyst containing nickel, molybdenum, titanium, phosphorous, alumina and synthetic clay (catalyst A, a catalyst for use in the process of the present invention) was prepared by the following general procedure:

- an aqueous solution comprising aluminum chloride, titanium tetrachloride, and acetic acid was prepared;
- titanium phosphate particles were caused to precipitate from said solution by combining said solution with a second aqueous solution containing phosphoric acid, resulting in a slurry containing said titanium phosphate particles;
- an aqueous nickel chloride solution was added to said slurry to form a nickel-containing mixture;
- aqueous solutions containing ammonia and ammonium molybdate were added to said mixture, to bring pH of the mixture to 4.0 to 4.5;
- an aqueous slurry of synthetic clay (described in Granquist U.S. Pat. No. 3,252,757) was added to said mixture;
- an aqueous solution containing ammonia was added to said mixture, causing further coprecipitation at a pH of 6 to 6.5 of soluble metals not previously precipitated;
- the resulting slurry was filtered to produce a filter cake, which was washed free of soluble ions;
- the catalyst was aged 12 hours in a steam atmosphere, dried at 250° F. overnight, and calcined at a high rate of dry air at a terminal temperature of 950° F.

The particle density of the catalyst was 1.5 g./cc.

## EXAMPLE 2

A catalyst containing nickel, molybdenum, titanium, phosphorus, fluoride and alumina (catalyst B, a catalyst for use in the process of the present invention) was prepared by the following general procedure:

- an aqueous solution comprising aluminum chloride, titanium tetrachloride, and acetic acid was prepared;
- titanium phosphate particles were caused to precipitate from said solution by combining said solution with a second aqueous solution containing phosphoric acid, resulting in a slurry containing said titanium phosphate particles;
- an aqueous nickel chloride solution was added to said slurry to form a nickel-containing mixture;
- aqueous solutions containing ammonia, molybdc oxide and sodium hydroxide were added to said mixture, causing coprecipitation at a pH of 6 to 6.5 of soluble metals not previously precipitated;
- ammonium fluoride was stirred into the mixture;
- the resulting slurry was filtered to produce a filter cake, which was washed free from soluble ions.
- The catalyst was dried in flowing air at 125° F. and calcined at a high rate of dry air at a terminal temperature of 950° F.

The particle density of the catalyst was 1.52 g./cc.

## EXAMPLE 3

A low-density catalyst containing nickel, molybdenum, titanium, phosphorus and alumina (catalyst C, a comparison catalyst) was prepared by the following general procedure:

- an aqueous solution comprising aluminum chloride, titanium tetrachloride, and acetic acids was prepared;
- titanium phosphate particles were caused to precipitate from said solution by combining said solution with a second aqueous solution containing phosphoric acid, resulting in a slurry containing said titanium phosphate particles;
- an aqueous nickel chloride solution was added to said slurry to form a nickel-containing mixture;

- d. aqueous solutions containing ammonia, molybdc oxide and sodium hydroxide were added to said mixture, causing coprecipitation at a pH of 6 to 6.5 of soluble metals not previously precipitated;
- e. the resulting slurry was filtered to produce a filter cake, which was washed free of soluble ions;
- f. the catalyst was dried at 125° F. and calcined in a sealed pan with no airflow. The calcination was conducted by heating directly to 400° F. and holding 3 hours while added water at 100 cc./hour. The temperature was adjusted to 700° F. and then held 2.5 hours at 900° F.
- The particle density of the catalyst was 1.18 g./cc.

## EXAMPLE 4

A catalyst containing nickel, tungsten, titanium, alumina and silica, but no phosphorus (catalyst D, a comparison catalyst) was prepared by suitable modification of the general procedure of example 1. The catalyst density was 1.74 g./cc.

## EXAMPLE 5

A catalyst containing nickel, molybdenum and alumina (catalyst E, a comparison catalyst) was prepared by the following general procedure:

- a. an aqueous solution comprising aluminum chloride, nickel chloride and acetic acid was prepared;
- b. an aqueous solution of molybdc acid and concentrated hydrochloric acid was added;
- c. an aqueous solution of ammonia was added to said mixture to raise the pH to 7, causing coprecipitation of soluble metals not previously precipitated;
- d. the resulting slurry was filtered to produce a filter cake, which was washed free of soluble ions;
- e. the catalyst was dried at 100° F. and calcined in flowing air which had been saturated with water at 70° F., with a terminal calcination temperature of 950° F.

The particle density of the catalyst was 1.70 g./cc. The nominal compositions of the catalysts are shown in table I.

TABLE I.—COMPOSITION OF CATALYSTS

| Example | Catalyst | Ni  | Mo | W  | Clay | F   | TiO <sub>2</sub> | P <sub>2</sub> O <sub>5</sub> | SiO <sub>2</sub> | Al <sub>2</sub> O <sub>3</sub> |
|---------|----------|-----|----|----|------|-----|------------------|-------------------------------|------------------|--------------------------------|
| 1.      | A        | 6.4 | 16 | —  | 20   | —   | 8                | 4                             | —                | 32                             |
| 2.      | B        | 8   | 20 | —  | —    | 4.5 | 10               | 5                             | —                | 40                             |
| 3.      | C        | 8   | 20 | —  | —    | —   | 10               | 6.5                           | —                | 43                             |
| 4.      | D        | 15  | —  | 20 | —    | —   | 5.6              | —                             | 19.5             | 30.5                           |
| 5.      | E        | 7.6 | 18 | —  | —    | —   | —                | —                             | 65.4             | —                              |

The catalysts of examples 1–5 were used to hydrogenate separate portions of a California light-cycle oil of the following description:

|                          |         |
|--------------------------|---------|
| Gravity, °API            | 22.3    |
| Aniline point, °F.       | 61.2    |
| Sulfur, wt. %            | 1.27    |
| Nitrogen, p.p.m.         | 2,140   |
| Aromatic content, LV%    | 60      |
| ASTM O-1160 Distillation |         |
| ST/5                     | 394/459 |
| 10/30                    | 475/504 |
| 50                       | 527     |
| 70/90                    | 549/580 |
| 95/EP                    | 593/627 |

The hydrogenation was accomplished in a reactor under the following conditions:

|                                                          |       |
|----------------------------------------------------------|-------|
| Total Pressure, p.s.i.g.                                 | 2,000 |
| Total hydrogen supply rate, SCF/bbl. of hydrocarbon feed | 5,000 |
| Liquid hourly space velocity, V.V./hour                  | 1.0   |
|                                                          |       |

The performances of the catalysts in this test are shown in table II. At these conditions, conventional platinum-alumina hydrogenating catalysts would be inoperable, due to the high-feed sulfur content.

The nominal activities at 725° of the several catalysts are shown in table III.

TABLE II.—HYDROGENATION OF AROMATICS IN LCO (60% AROMATICS CONTENT)

| Catalyst | LHSV <sub>v</sub> | LHSV <sub>w</sub> | Catalyst temp., °F. | Activity       |                |                |                |
|----------|-------------------|-------------------|---------------------|----------------|----------------|----------------|----------------|
|          |                   |                   |                     | A <sub>e</sub> | A <sub>d</sub> | k <sub>v</sub> | k <sub>w</sub> |
| 5        | A                 | 0.98              | 700                 | 1.5            | 17.5           | 1.27           | 1.34           |
|          |                   | 0.99              | 700                 | 1.5            | 18.1           | 1.28           | 1.34           |
|          |                   | 1.00              | 700                 | 1.5            | 21.5           | 1.08           | 1.17           |
| 10       | B                 | 1.00              | 700                 | 1.5            | 17.7           | 1.28           | 1.33           |
|          |                   | 0.99              | 720                 | 2.5            | 14.0           | 1.60           | 1.66           |
|          |                   | 0.99              | 720                 | 2.5            | 14.5           | 1.56           | 1.61           |
| 15       | C                 | 1.04              | 725                 | 2.7            | 17.2           | 1.42           | 1.97           |
|          |                   | 1.02              | 725                 | 2.7            | 17.0           | 1.42           | 1.93           |
|          | D                 | 1.02              | 725                 | 2.7            | 17.1           | 1.24           | 1.15           |
| 20       |                   | 1.02              | 725                 | 2.7            | 17.4           | 1.23           | 1.13           |
|          |                   | 0.97              | 725                 | 2.7            | 19.8           | 1.04           | 1.01           |
|          |                   | 1.04              | 725                 | 2.7            | 17.4           | 1.24           | 1.15           |
| 25       | E                 | 1.01              | 720                 | 2.5            | 23.6           | 1.02           | 1.03           |
|          |                   | —                 | —                   | —              | —              | —              | —              |
|          |                   | —                 | —                   | —              | —              | —              | —              |

TABLE III NOMINAL ACTIVITIES AT 725° F.

|                                    | Activity (weight basis) | Activity (volume basis) | Particle Density |
|------------------------------------|-------------------------|-------------------------|------------------|
| Catalysts of the Present Invention |                         |                         |                  |
| Catalyst A                         | 1.75                    | 1.70                    | 1.50             |
| Catalyst B                         | 1.75                    | 1.70                    | 1.52             |
| Prior art catalysts                |                         |                         |                  |
| Catalyst C                         | 1.75                    | 1.10                    | 1.18             |
| Catalyst D                         | 1.05                    | 1.10                    | 1.74             |
| Catalyst E                         | 1.00                    | 1.00                    | 1.70             |

It is apparent that catalysts A and B, catalysts of the present invention, have a hydrogenation activity substantially above that of the other catalysts of the above tabulation. Catalyst C had a composition which is appropriate, but is density and its activity on a volume basis are too low, since it was improperly calcined. A change in the calcination procedure as discussed herein will raise the density and bring the volumetric activity up to the 1.70 level of catalysts A and B. Catalyst D, containing tungsten instead of molybdenum and without phosphorus pen-

toxide, has low activity, even though the catalyst density is high, catalyst E, which does not contain titanium phosphate or zirconium phosphate, has sufficient density but still has low activity.

## CONCLUSIONS

From the foregoing it may be seen that the process of the present invention is effective for accomplishing a given amount of aromatics hydrogenation of a lower temperature than is possible with certain processes using different catalysts. It also may be seen that the process of the present invention is effective for accomplishing a greater amount of hydrogenation at a given temperature, for longer periods of time, than is possible with certain processes using different catalysts. It is further may be seen that the catalyst used in the process of the present invention, compared with the conventional prior art aromatics hydrogenation catalysts, does not require the use of costly group VIII noble metals, and is sulfur- and nitrogen-tolerant.

What is claimed is:

1. An aromatics hydrogenation process which comprises contacting an aromatics-containing hydrocarbon feedstock under aromatics hydrogenation conditions with hydrogen and a catalyst comprising alumina, 0.5 to 20 weight percent synthetic clay, a component selected from nickel and compounds thereof and cobalt and compounds thereof, a component selected from molybdenum and compounds thereof, and a component selected from titanium phosphate and zir-

conium phosphate, said catalyst having a particle density greater than 1.4 g./cc., and said catalyst containing no noble metal and also containing no silica other than combined silica said synthetic clay.

2. A process as in claim 1, wherein said catalyst has a bulk density greater than 1.5 g./cc.

3. A process as in claim 1, wherein said feedstock contains sulfur in excess of 200 p.p.m.